

# UNITED STATES PATENT OFFICE.

HARRY SCHMIDT, OF COLOGNE, GERMANY.

## PROCESS FOR PRODUCING PORELESS AND WELL-ADHERING ELECTRODEPOSITS.

No. 880,405.

Specification of Letters Patent.

Patented Feb. 25, 1908.

Application filed August 7, 1907. Serial No. 387,628.

*To all whom it may concern:*

Be it known that I, HARRY SCHMIDT, a subject of the King of Prussia, residing at Cologne-on-the-Rhine, in the Kingdom of Prussia and German Empire, have invented a new and useful Improvement in Processes for Producing Poreless and Well-Adhering Electrodeposits, of which the following is a specification.

10 Electrodeposited metal does not generally afford sufficient protection against chemical influences; because, unless extremely thick, it contains innumerable fine pores, through which the metal to be protected can be attacked. In many cases chemical action is assisted by decomposing local electric currents, which circulate between the base metal and the electrodeposit when moist. In order to afford an effective protection of 20 the base metal, the pores in the electrodeposit must therefore be closed. This is effected according to the present invention by first coating—by any suitable process such as electroplating or dipping—the metal 25 to be electroplated, with a metal or alloy having a lower melting point than the final electrodeposit, whereupon it is provided

with the electrodeposit, and, after drying and cleaning the surface, is then subjected to a temperature higher than the melting point 30 of the intermediate coating. This coating accordingly melts, and becomes intimately united with both the base metal and electrodeposit, simultaneously filling out the pores contained in the latter, without injuring said 35 base metal and electrodeposit.

What I claim and desire to secure by Letters Patent is:—

The process for producing poreless and well adhering electrodeposits, which consists in first providing the metal to be electroplated with a coating of a metal or alloy which melts at a lower temperature than the final electrodeposit, in then electrolytically 40 depositing the final coating, and in melting 45 the intermediate coating, substantially as, and for the purpose, set forth.

In testimony whereof I have signed my name to this specification in the presence of two subscribing witnesses.

HARRY SCHMIDT.

Witnesses:

LOUIS VANDORN,  
M. KNEPPERS.